

## UNITED STATES PATENT OFFICE

2,597,504

METHOD OF EXTRACTING URANIUM FROM  
BITUMINOUS SHALES AND SHALE CULM  
CONTAINING URANIUMMarkus Larsson, Stockholm, Sweden, assignor to  
Frans Georg Liljenroth, Stockholm, Sweden

No Drawing. Application December 3, 1948, Serial No. 63,441. In Sweden December 4, 1947

4 Claims. (Cl. 23—14.5)

1

Deposits of bituminous shales contain in many cases a small percentage of uranium. Particularly in the mineral called shale culm occurring in bituminous shales as balls or lenses rich in organic matters the percentage of uranium is essentially higher than in the bituminous shale per se. For instance the percentage of uranium in bituminous shales can amount to 0.02 to 0.03% by weight while the percentage of uranium in the shale culm may be for instance 0.4 to 0.5% by weight. As the percentage of combustible organic matter in the shale culm is rather high the ash from such culm can contain up to 2 to 2.5% by weight of uranium.

It has already been proposed to leach ashes from shale culm with a solution of sodium carbonate in order to extract uranium, radium and other valuable constituents. The result was, however, not satisfactory as only about  $\frac{1}{5}$  to  $\frac{1}{4}$  of the total percentage of uranium in the ash could be recovered in such manner. In leaching ashes from bituminous shale containing uranium with a solution of sodium carbonate the result will likewise be unsatisfactory as the chief part of the uranium will remain in an insoluble state in the ash.

This invention relates to an improved method of extracting uranium from bituminous shales and shale culm containing uranium by means of a solution of alkali carbonate and consists chiefly in this that the shale or the shale culm is leached in its natural state, i. e. without a preceding coking or combustion of the raw material to ash. In such leaching operation it is not necessary to grind the raw material to a fine powder in as much as a satisfactory extraction of the uranium can be performed, if the raw material is crushed to a grain size of about 0.25 to 0.15 mm.

In the leaching of the raw material in its natural state with a solution of alkali carbonate the astonishing effect is attained that the yield of uranium will be essentially higher than in leaching ashes from said raw material though the quantity of raw material in the former case is essentially larger than in the latter case, for instance in leaching shale culm in natural state about 4 to 5 times larger than in leaching ashes from the culm.

It has been found that the extraction of the uranium is facilitated and improved if the raw material before or after its mixing with the solution of alkali carbonate is subjected to the oxidizing action of air or a gas rich in oxygen at a temperature slightly above room tempera-

2

ture, for instance in such manner, that air or a gas rich in oxygen is blown through a sludge of the raw material and a solution of an alkali carbonate, or in such manner, that the raw material is moistened with a solution of alkali carbonate of a suitable concentration whereupon air or gas rich in oxygen is conducted through the moist though still porous mass.

In such oxidizing step a maximum effect is obtained by using air or a gas rich in oxygen at a temperature of about 25 to 35° C. It is essential that the oxidizing is carried out at a moderate temperature in as much as otherwise the organic substance in the raw material also would be oxidized to a considerable extent and be dissolved in the alkali carbonate solution.

In leaching the raw material without a preceding oxidizing I have found that an increase of the leaching temperature does not essentially increase the yield of uranium until the boiling point of the solution is reached, but at the boiling temperature the yield is highly increased.

In extracting shale culm with a solution of alkali carbonate a higher yield of uranium is obtained at boiling temperature without oxidizing than by oxidizing without using a high temperature in the extraction process, but the best result will be obtained if the raw material is first oxidized at a temperature of about 25 to 35° C. and then extracted by means of a solution of alkali carbonate at the boiling point of the latter.

In order to obtain a good yield a rather concentrated solution of alkali carbonate should be used. When bituminous shales containing sulphuric acid either as free acid or as sulphates are treated the alkali carbonate is partly converted into alkali sulphate. In the oxidizing step also the sulphides possibly present in the raw material are oxidized to  $SO_2$  and possibly also to  $SO_3$  which also convert a part of the alkali carbonate to alkali sulphite and alkali sulphate respectively. The solution separated from the leached raw material can preferably be used repeatedly in leaching fresh quantities of the raw material in which case, however, also fresh quantities of alkali carbonate should be added to the solution so as to maintain its content of alkali carbonate substantially constant.

By using the leaching solution repeatedly its content of uranium is successively increased. When the uranium has reached a suitable concentration in the solution the latter is drawn off whereupon the uranium is precipitated, for instance by neutralizing the alkali carbonate with

sulphuric acid, whereby the uranium is caused to precipitate as alkali diuranate. The solution separated from the precipitate and containing chiefly alkali sulphite and alkali sulphate may be evaporated and the solid salts recovered be converted in well-known manner into alkali carbonate for renewed use in the process.

As alkali carbonate preferably sodium carbonate,  $Na_2CO_3$ , is used but also potassium carbonate or ammonium carbonate or bicarbonates of the alkalis may be used. Sodium carbonate is, of course, to be preferred as it is the cheapest alkali carbonate. When not otherwise stated I use in the specification and the claims the expression "alkali carbonate" in a sense including the normal alkali carbonate,  $MgCO_3$  as well as the alkali bicarbonate,  $MgHCO_3$ .

Instead of oxidizing the raw material mixed with the alkali carbonate it is possible to oxidize the raw material before the alkali carbonate solution is added.

I have found that in carrying out the process with some bituminous shales containing uranium the yield of uranium will be low even if the raw material is oxidized as above described and then extracted with a solution of alkali carbonate at the boiling temperature of the latter. In such case the yield can be essentially improved by performing the leaching operation in a closed apparatus at an over-pressure and at a correspondingly high temperature above 100° C. In such case it is not always necessary to oxidize the raw material. It is also to be noted that in such case good results are obtained not only when using a solution of normal alkali carbonate as leaching agent but also when a solution of alkali bicarbonate or a solution containing a mixture of alkali carbonate and alkali bicarbonate is used. When alkali bicarbonate is used as leaching agent carbon dioxide is developed during the high extraction temperature used, which causes an elevation of the pressure in the closed apparatus. When using temperatures above 200° C. in the extraction process also the silicic acid of the raw material is dissolved by the normal alkali carbonate to a considerable extent. Said inconveniences are, however, substantially avoided by using as leaching agent a solution containing alkali bicarbonate up to 50% of the total quantity of alkali carbonate. I have found that in such case the development of carbon dioxide also at high temperatures as well as the dissolving of silicic acid are essentially reduced. When leaching the raw material with a solution containing normal alkali carbonate as well as alkali bicarbonate at high pressures and high temperatures the yield of uranium is also improved in comparison with a leaching under the same conditions with a solution containing normal alkali carbonate alone.

#### Examples

I. 1 kg. of bituminous shale containing uranium and ground to such grain size that 99% thereof passed through a sieve with 25 mm. meshes was mixed with 1 l. of a 10% solution of sodium carbonate whereupon oxygen was supplied to the mixture at a temperature of about 25° C. When about 1.5 l. oxygen had been absorbed the solid matters were separated by filtering and washing. The clear solution obtained contained .24 g. of uranium oxide ( $U_3O_8$ ) which could be recovered as sodium uranate by neutralizing with sulphuric acid.

II. 1 kg. of the same bituminous shale as in Example I was mixed with 1 l. of a 10% solution

of sodium carbonate whereupon the sludge was heated to the boiling point while stirring during about 1 hour. The solution separated from the sludge contained .24 g. of uranium oxide ( $U_3O_8$ ).

III. 1 kg. of the same bituminous shale as in Example I was mixed with 1 l. of a 10% solution of sodium carbonate whereupon the sludge was oxidized as in Example I and then boiled while stirring during 30 minutes. The solution separated from the sludge contained .27 g. of  $U_3O_8$ .

IV. 1 kg. of the same shale as in Example I was mixed with 2 l. of a 10% solution of sodium carbonate whereupon air was blown through the sludge while stirring during 1½ to 2 hours. The solution separated from the sludge contained .245 of  $U_3O_8$ .

V. 1 kg. of another sample of bituminous shale ground to the same fineness as in Example I was boiled while stirring together with 1 l. of a 10% solution of sodium carbonate. The clear solution separated from the sludge contained .13 g. of  $U_3O_8$ .

VI. .4 kg. of the same shale as in Example V was mixed with a solution of 8 g. of  $NaOH$  and 10 g. of  $Na_2CO_3$  in about 70 cc. of water. The moist mass was placed in a U-shaped tube through which oxygen was conducted. The mass was then mixed with 400 cc. of water and sodium carbonate was added until a concentration of 10%. The mixture was then heated to the boiling point while stirring in about 1 hour. The solution separated contained .17 g. of  $U_3O_8$ .

VII. .5 kg. of a shale culm ground to such grain size that 99% passed through a sieve with .15 mm. meshes was mixed with 1 l. of a 10% solution of sodium carbonate whereupon the mixture was heated to the boiling point while stirring during about 2 hours. The solution separated from the sludge contained 1.725 g. of  $U_3O_8$ , corresponding to an output of about 78%.

VIII. .5 kg. of the same shale culm as in Example VII was mixed with 1 kg. of a 10% solution of sodium carbonate whereupon the mixture was first oxidized by means of oxygen at 30° C. and then heated to the boiling point while stirring during 2 hours. The solution separated from the sludge contained 1.962 g. of  $U_3O_8$ , corresponding to an output about 90%.

IX. 1 kg. of a bituminous shale ground to such grain size that 90% thereof were less than 0.15 mm. was mixed with 1.4 l. of a 10% solution of sodium carbonate whereupon the sludge was heated to 50° C. and then shaken in an atmosphere of oxygen until 2 l. of the oxygen had been absorbed. The sludge was then heated to the boiling point of the solution while stirring in about 2 hours. The solution contained .08 g. of  $U_3O_8$ .

X. This test was carried out with the same shale as in Example IX but at an overpressure and a correspondingly elevated temperature. 1 kg. of the shale was mixed with 1.4 l. of a 10% solution of sodium carbonate whereupon the sludge was heated to a temperature of about 160° C. at an overpressure of 5.5 atmospheres during 2 hours while stirring. After filtering and washing the clear solution obtained contained .18 g. of uranium oxide ( $U_3O_8$ ).

I claim:

1. Method of extracting uranium from bituminous shale containing uranium, which comprises preparing a suspension of the shale in its natural chemical state in a solution of alkali carbonate, blowing a gas containing free oxygen

through said suspension and then separating the extract from the solid matters.

2. Method of extracting uranium from bituminous shale containing uranium, which comprises preparing a suspension of the shale in its natural chemical state in a solution of alkali carbonate, blowing a gas containing free oxygen through said suspension while maintaining the suspension at a temperature of 25 to 33° C., and then separating the extract from the solid matters.

3. Method of extracting uranium from bituminous shale containing uranium, which comprises preparing a suspension of the shale in its natural chemical state in a solution of alkali carbonate, blowing a gas containing free oxygen through said suspension, then heating the suspension to a temperature of at least 100° C., and finally separating the solution from the solid matters.

4. Method of extracting uranium from bituminous shale containing uranium, which comprises preparing a suspension of the shale in

its natural chemical state in a solution of alkali carbonate, blowing a gas containing free oxygen through said suspension, separating the extract from the solid matters, adding alkali carbonate to the extract and returning the extract into the process for the treatment of further quantities of the raw material.

MARKUS LARSSON.

#### REFERENCES CITED

The following references are of record in the file of this patent:

#### UNITED STATES PATENTS

| Number    | Name     | Date           |
|-----------|----------|----------------|
| 1,429,550 | Vogt     | Sept. 19, 1922 |
| 1,438,357 | Bleecker | Dec. 12, 1922  |
| 1,999,807 | Gibbs    | Apr. 30, 1935  |

#### OTHER REFERENCES

20 Mellor, Inorganic and Theoretical Chemistry, volume 12, page 8 (1932). Published by Longmans, Green and Company, London.